

Sept. 14, 1965

H. D. PORTER ET AL

3,206,313

CHEMICALLY SENSITIZED EMULSIONS HAVING LOW SURFACE  
SENSITIVITY AND HIGH INTERNAL SENSITIVITY

Filed May 15, 1961

MIDDLE RANGE RECIPROCITY CHARACTERISTICS OF  
CG and CONTROL (CORE) EMULSIONS



Henry D. Porter  
Thomas H. James  
Wesley G. Lowe  
INVENTORS

BY *R. Frank Smith*  
*Lawrence H. Willis*  
ATTORNEYS

3,206,313

**CHEMICALLY SENSITIZED EMULSIONS HAVING LOW SURFACE SENSITIVITY AND HIGH INTERNAL SENSITIVITY**

Henry D. Porter, Thomas H. James, and Wesley G. Lowe, Rochester, N.Y., assignors to Eastman Kodak Company, Rochester, N.Y., a corporation of New Jersey

Filed May 15, 1961, Ser. No. 110,109  
13 Claims. (Cl. 96—108)

This invention relates to photographic elements and photographic emulsions having improved sensitivity, and more particularly, to photographic layers comprising photographic silver halide emulsions which have high internal sensitivity induced by chemical sensitization and low surface sensitivity.

Emulsions having high internal sensitivity, but low surface sensitivity, have been previously described in the photographic art by Davey and Knott in U.S. Patent 2,592,250, issued April 8, 1952. However, it has not been previously possible to increase substantially the internal sensitivity of these emulsions by chemical sensitizing. Chemical sensitization as conventionally carried out, for example, by sulfur or gold sensitization, increases the surface sensitivity of the emulsions, but has little or no effect upon the internal sensitivity. In fact, in many cases, the internal sensitivity and gamma decrease during chemical sensitization, while the surface sensitivity and gamma are increased.

We have now found a new method which makes possible the preparation of photographic silver halide emulsions having high internal sensitivity induced by chemical sensitization, but which exhibit low surface sensitivity.

It is, therefore, an object of our invention to provide photographic silver halide emulsions containing silver halide grains which have high internal sensitivity induced by chemical sensitization, but which exhibit low surface sensitivity. Another object of our invention is to protect the high internal sensitivity of the photographic silver halide emulsion prepared according to our invention. Another object is to decrease the reciprocity failure exhibited by photographic silver halide emulsions prepared according to prior art methods which exhibit high internal sensitivity, but low surface sensitivity. Still another object is to reduce the desensitization of many spectral sensitizing dyes in the blue region of the spectrum when these dyes are used to extend the spectral range of silver halide emulsions. Other objects will become apparent from a consideration of the following description and examples.

According to our invention, we have found that the above objects can be realized by blending a very fine grain silver halide emulsion with a chemically sensitized emulsion having considerably larger average grain distribution and holding this mixture for a sufficient time to produce a substantially homogeneous grain size distribution. When these emulsions are freshly blended, the composite emulsion shows conventional behavior, high surface speed and fog. However, on holding the composite emulsion for a suitable length of time (generally several hours) at a suitable temperature, the blend is found to alter its characteristics, giving rise to a composite emulsion which exhibits very low surface speed and fog, but very high internal speed. The amount of internal fog obtained can be controlled by the amount of surface fog obtained in the finish of the coarser-grained component of the blend.

It is evident that the preparation of the novel internally-sensitized emulsions of our invention involves two discrete components. The coarser-grained component can be termed the core, for it appears that during the afore-mentioned period of holding, a ripening process

occurs during which the finer-grained component partially dissolves and recrystallizes upon the surface of the coarser-grained silver halide. The original surface sensitivity and fog specks of the coarser-grained silver halide, or the "core" grains are thus buried, causing them to behave as internal specks. The finer-grained silver halide can be termed the "shell" because it appears that these grains dissolve and recrystallize upon the surface of the core emulsion.

- 10 The core emulsions used in our invention comprise those which, when examined according to normal photographic testing techniques by coating a test portion of the emulsion on a transparent support, exposing to a light intensity scale for a fixed time between 0.01 and 1 second and development for 6 minutes at 68° F. in Developer A, as hereinafter defined, have a sensitivity greater than the sensitivity of an identical test portion of the same emulsion (measured at a density of 0.1 above fog), which has been exposed in the same way, bleached 5 minutes in an aqueous 0.3 percent potassium ferricyanide solution at 65° F., and developed for 5 minutes at 65° F., in Developer B, as hereinafter defined. Developer A is the usual type of surface image developer and Developer B is an internal developer having high silver halide solvent activity. The degree of internal sensitivity of the surface image emulsions is not particularly critical. The surface image emulsion can have relatively little internal sensitivity, or it may have a fair amount of internal sensitivity. Suitable surface image silver halide emulsions can be any of the conventional silver halide emulsions, although we have found that silver bromide emulsions containing a relatively high content of bromide are particularly useful. These emulsions can contain up to about 10 percent of another silver halide, such as silver iodide. Silver bromide and silver bromoiodide emulsions are particularly useful in our invention. Such emulsions have been previously described by Trivelli and Smith in "The Photographic Journal," vol. LXXX, July 1940 (pages 285-288).
- 20 Before blending with the shell emulsions, the core emulsions are first chemically sensitized by means which have been previously described in the prior art. By chemical sensitization, we mean sensitization of the type described by Antoine Hautot and Henri Saubenier in "Science et Industries Photographiques," vol. XXVIII, January 1957, pages 1-23 and January 1957, pages 57-65. Such chemical sensitization includes three major classes, viz., gold or noble metal sensitization, sulfur sensitization, such as by a labile sulfur compound, and reduction sensitization, i.e., treatment of the silver halide with a strong reducing agent which does not fog appreciably the silver halide but introduces small specks of metallic silver into the silver halide crystal or grain.
- 30 The core emulsions can be chemically sensitized by any of the accepted procedures. The core emulsions can be digested with naturally active gelatin, or sulfur compounds can be added, such as those described in Sheppard U.S. Patent 1,574,944, issued March 2, 1926, Sheppard et al. U.S. Patent 1,623,499, issued April 5, 1927, and 40 Sheppard et al. U.S. Patent 2,410,689, issued November 5, 1946.
- 40 The core emulsions can also be treated with salts of the noble metals, such as ruthenium, rhodium, palladium, iridium, and platinum. Representative compounds are 45 ammonium chloropalladate, potassium chloroplatinate, and sodium chloropalladite, which are used for sensitizing in amounts below that which produces any substantial fog inhibition, as described in Smith and Trivelli U.S. Patent 2,448,060, issued August 31, 1948, and as 50 antifoggants in higher amounts, as described in Trivelli and Smith U.S. Patents 2,566,245, issued August 28, 1951 and 2,566,263, issued August 28, 1951.

The core emulsions can also be chemically sensitized with gold salts as described in Waller et al. U.S. Patent 2,399,083, issued April 23, 1946, and Damschroder et al. U.S. Patent 2,642,361, issued June 16, 1953. Suitable compounds are potassium chloroaurite, potassium aurithiocyanate, potassium chloroaurate, auric trichloride and 2-aurosulfobenzothiazole methochloride.

The core emulsions can also be chemically sensitized with reducing agents, such as stannous salts (Carroll U.S. Patent 2,487,850, issued November 15, 1949), polyamines, such as diethylene triamine (Lowe and Jones U.S. Patent 2,518,698, issued August 15, 1950), polyamines, such as spermine (Lowe and Allen U.S. Patent 2,521,925, issued September 12, 1950), or bis( $\beta$ -aminoethyl)sulfide and its water - soluble salts (Lowe and Jones U.S. Patent 2,521,926, issued September 12, 1950).

The core emulsions can also be optically sensitized with cyanine and merocyanine dyes, such as those described in Brooker U.S. Patents 1,846,301, issued February 23, 1932; 1,846,302, issued February 23, 1932; and 1,942,854, issued January 9, 1934; White U.S. Patent 1,990,507, issued February 12, 1935; Brooker and White U.S. Patents 2,112,140, issued March 22, 1938; 2,165,338, issued July 11, 1939; 2,493,747, issued January 10, 1950 and 2,739,964, issued March 27, 1956; Brooker and Keyes U.S. Patent 2,493,748, issued January 10, 1950; Sprague U.S. Patents 2,503,776, issued April 11, 1950 and 2,519,001, issued August 15, 1950; Heseltine and Brooker U.S. Patent 2,666,761, issued January 19, 1954; Heseltine U.S. Patent 2,734,900, issued February 14, 1956; VanLare U.S. Patent 2,739,149, issued March 20, 1956; and Kodak Limited British Patent 450,958, accepted July 15, 1936.

The core emulsions can also contain speed increasing compounds of the quaternary ammonium type of Carroll U.S. Patent 2,271,623, issued February 3, 1942; Carroll and Allen U.S. Patent 2,288,226, issued June 30, 1942; and Carroll and Spence U.S. Patent 2,334,864, issued November 23, 1943; or the polyethylene glycol type of Carroll and Beach U.S. Patent 2,708,162, issued May 10, 1955; or the quaternary ammonium salts and polyethylene glycols of Piper U.S. Patent 2,886,437, issued May 12, 1959; as well as the thiopolymers of Graham and Sagal U.S. application Serial No. 779,839, filed December 12, 1958 (now U.S. Patent 3,046,129, issued July 24, 1962) and the Dann and Chechak U.S. application Serial No. 779,874, filed December 12, 1958 (now U.S. Patent 3,046,134, issued July 24, 1962).

The shell emulsions useful in our invention can be prepared according to techniques which have been previously described in the prior art. Methods for preparing such emulsions have been previously described by Trivelli and Smith in "The Photographic Journal," vol. LXXIX, May 1939, pages 330-338. While any of the usual silver halides, such as silver chlorobromide, and the like, can be used in the shell emulsions, particularly useful results have been obtained with silver bromide emulsions, particularly silver bromide emulsions containing at least 90 mole percent of silver bromide. Other halides, up to about 10 percent, can be used with the silver bromide emulsions. Silver bromide and silver bromoiodide emulsions (e.g., silver bromoiodide emulsions containing up to about 10 mole percent of iodide) have been found to be particularly useful in preparing the shell emulsions of our invention. Generally, the shell emulsions are chemically unsensitized, although for special applications it may be desired to sensitize these emulsions according to the technique described above for the core emulsions.

In order to obtain the useful effects illustrated below, it is important that the grain size distribution of the shell emulsions be such that the average grain size is not greater than  $0.4\mu$ , and preferably about  $0.1\mu$ . The average grain size distribution of the core emulsions should be such that the silver halide grain size has a diameter greater than about  $0.8\mu$  (e.g., 0.8 to about  $1.5\mu$ ).

In general, we have found that particularly useful re-

sults can be obtained by blending about 0.25 to about 8.0 molar equivalents of the shell emulsion per molar equivalent of the core or surface-sensitive emulsion. When these blends are held for several hours, usually for about 24 hours, at room temperature, the shell grains dissolve and deposit upon the surface of the core grains so that the resulting composite emulsion shows very high internal sensitivity, but very low surface sensitivity. Also, the resulting composite emulsion, which can be termed a "covered grain" emulsion, contains a population of silver halide grains which are more or less uniform in grain-size distribution, as contrasted with other emulsion blends which contain at least two types of silver halide grains, which are separate and distinct in their physical and, frequently, photographic properties.

The following developing solutions are used in the characterization of the silver halide emulsions described in this application.

|    |                                |           |
|----|--------------------------------|-----------|
|    |                                | A         |
| 20 | N-methyl-p-aminophenol sulfate | grams 2.5 |
|    | Ascorbic acid                  | do 10     |
|    | Potassium metaborate           | do 35     |
|    | Potassium bromide              | do 1      |
| 25 | Water to 1 liter.              |           |
|    | pH                             | 9.6       |

|    |                                |           |
|----|--------------------------------|-----------|
|    |                                | B         |
| 30 | N-methyl-p-aminophenol sulfate | grams 2.0 |
|    | Sodium sulfite, desiccated     | do 90     |
|    | Hydroquinone                   | do 8.0    |
|    | Sodium carbonate, monohydrate  | do 52.5   |
|    | Potassium bromide              | do 5      |
| 35 | Sodium thiosulfate             | do 10     |
|    | Water to 1 liter.              |           |

|    |                                |           |
|----|--------------------------------|-----------|
|    |                                | C         |
| 40 | N-methyl-p-aminophenol sulfate | grams 2.5 |
|    | Sodium sulfite, desiccated     | do 30     |
|    | Hydroquinone                   | do 2.5    |
|    | Sodium metaborate              | do 10     |
|    | Potassium bromide              | do 0.5    |
| 45 | Water to 1 liter.              |           |

|    |                                |           |
|----|--------------------------------|-----------|
|    |                                | D         |
| 45 | N-methyl-p-aminophenol sulfate | grams 2.2 |
|    | Hydroquinone                   | do 8.8    |
|    | Sodium sulfite, desiccated     | do 72     |
|    | Sodium carbonate, crystalline  | do 130    |
|    | Potassium bromide              | do 4.0    |
| 50 | Potassium iodide               | do 0.5    |
|    | Water to make 1 liter.         |           |

Ordinary photographic silver halide emulsions which have been chemically sensitized according to methods which have been previously described in the prior art tend to lose a good deal of their sensitivity upon storage, usually as a result of chemical interaction with the environment. On the other hand, the covered grain emulsions of our invention do not exhibit to such a marked degree the loss of their chemical sensitivity, since the internal chemical sensitivity centers are covered by a layer of protective silver halide. Moreover, these covered grain emulsions retain their high spectral sensitivity and do not exhibit the marked blue desensitization which is characteristic of many prior art spectrally-sensitized silver halide emulsions. Moreover, the covered grain emulsions of our invention have much improved reciprocity failure characteristics as hereinafter shown. The following examples will serve to illustrate the improved photographic properties of the covered grain emulsion of our invention.

#### EXAMPLE 1

One part of an ordinary photographic gelatino-silver bromoiodide emulsion which had been sulfur-sensitized with a labile sulfur compound, e.g., allylthiourea, con-

taining about 2 mole percent iodide and having an average grain size of about  $1.0\mu$  diameter was blended with 1 part of a very fine grain, unsensitized gelatino-silver-bromoiodide emulsion containing about 2 mole percent iodide and having an average grain size of about  $0.1\mu$  diameter. Another 1 part aliquot portion of the sulfur-sensitized emulsion was also blended with 1 part of an ordinary gelatino-silver-bromoiodide emulsion (unsensitized) containing about 2 mole percent iodide and hav-

5 allowed to stand for 24 hours at  $40^\circ$  F. and then coated on a cellulose acetate film support. A third sample of the blend was coated fresh on cellulose acetate film support. The three samples were then separately exposed and processed exactly as described in Example 1 above, except that the surface development was for 5 minutes in Developer C and internal development was for 5 minutes in Developer B. The results obtained are summarized in the following table.

Table II

| Coating Number | Holding Time Before Coating   | Surface Development |          |      | Internal Development |          |      |
|----------------|-------------------------------|---------------------|----------|------|----------------------|----------|------|
|                |                               | Relative Speed      | $\gamma$ | Fog  | Relative Speed       | $\gamma$ | Fog  |
| (f)-----       | Fresh-----                    | 100                 | 0.68     | 0.11 | 9.4                  | 0.44     | 0.20 |
| (g)-----       | 24 hrs. at $70^\circ$ F.----- | <1.0                | <0.1     | 0.05 | 209                  | 0.70     | 0.25 |
| (h)-----       | 24 hrs. at $40^\circ$ F.----- | 58                  | 0.45     | 0.08 | 42                   | 0.45     | 0.22 |

ing an average grain size of about  $0.4\mu$  diameter. The 2 blends were separately held at room temperature for several hours and then coated upon ordinary cellulose acetate film support. Separate samples of each emulsion component of the blends were also coated on separate cellulose acetate film supports. The dried samples of coating were then exposed for 1 second to a 500-watt,  $3000^\circ$  K. light source on an Eastman Ib sensitometer and developed for 12 minutes in a surface developer having the composition given above as Developer A. Separate strips of each coating were then exposed in an identical manner, bleached for 5 minutes at  $70^\circ$  F. in an aqueous solution containing 3 grams of potassium ferricyanide per liter of water and buffered to a pH of 5.0 with acetic acid and sodium acetate, rinsed and dried. The strips were then developed for 10 minutes in Developer B. The following results were obtained.

Table I

| Coating Number | Emulsion Type                                  | 12' In A Surface Developer (A) |          |     | 10' In An Internal Developer (B) |          |     |
|----------------|------------------------------------------------|--------------------------------|----------|-----|----------------------------------|----------|-----|
|                |                                                | Relative Speed                 | $\gamma$ | Fog | Relative Speed                   | $\gamma$ | Fog |
| (a)-----       | Sensitized-----                                | 100                            | 1.2      | .05 | 30                               | .6       | .01 |
| (b)-----       | Unsensitized $0.4\mu$ average grain size.----- | 1.59                           | 2.1      | .01 | 1.6                              | .5       | .01 |
| (c)-----       | Unsensitized $0.1\mu$ average grain size.----- | <.032                          | 0.0      | .01 | <.032                            | 0.0      | .00 |
| (d)-----       | 50-50 Blend of (a) plus (b).-----              | 69                             | 1.13     | .07 | 28                               | 1.1      | .03 |
| (e)-----       | 50-50 Blend of (a) plus (c).-----              | .8                             | .09      | .01 | 100                              | 1.35     | .09 |

EXAMPLE 2

A core emulsion comprising an ordinary photographic gelatino-silver-bromoiodide emulsion which had been sulfur-sensitized with a labile sulfur compound, e.g., allylthiourea, and gold-sensitized with a water-soluble gold salt, e.g., auric trichloride was mixed (50-50 blend) with an unsensitized shell emulsion containing about 1 mole percent silver iodide and 99 percent silver bromide. A sample of the blend was then allowed to stand for 24 hours at  $70^\circ$  F., and then coated on an ordinary cellulose acetate film support. A second sample of the blend was

55 the fine-grained emulsion (shell) could no longer be seen upon microscopic examination. The samples were then coated on ordinary cellulose acetate film support, dried, and exposed as described in Example 1 above. Strips of each sample were then developed in Developer 60 B (except that it contained no thiosulfate) for 5 minutes and separate strips were subjected to total development for 5 minutes in Developer D. The following results were obtained. (In total development the exposed emulsion sample is directly developed without "bleaching" off the surface latent image.)

Table III

| Coating  | Mole ratio of Emulsions Large/small | Ripening Time | "Surface" Development |       |      | "Total" Development |       |      |
|----------|-------------------------------------|---------------|-----------------------|-------|------|---------------------|-------|------|
|          |                                     |               | Relative Speed        | Gamma | Fog  | Relative Speed      | Gamma | Fog  |
| (i)----- | All large (core)-----               | 60 min-----   | 112                   | 1.79  | 0.16 | 100                 | 1.62  | 0.15 |
| (j)----- | 4:1-----                            | 60 min-----   | 1.1                   | 0.44  | 0.06 | 73                  | 1.10  | 0.68 |
| (k)----- | 2:1-----                            | 90 min-----   | Slight image          |       |      | 97                  | 1.12  | 0.70 |

7  
EXAMPLE 4

A high speed gelatino-silver-bromoiodide emulsion containing 1.7 mole percent of iodide and having an average grain size of about  $0.8\mu$  diameter was blended in the amounts shown below with a fine-grained gelatino-silver-bromoiodide emulsion as illustrated in Example 3 above, using 10.8 grams per silver mole of potassium bromide in the emulsion blends to accelerate digestion. The samples were then coated on cellulose acetate film support and dried. The samples were then exposed in an intensity scale sensitometer as described in Example 1 and strips of each sample were subjected to surface development for 5 minutes in Developer C. Strips of each sample were also subjected to total development for 5 minutes in Developer D. The following results were obtained.

5  
10  
15

Table IV

| Coating   | Mole Ratio, large/small | Hold Time     | KBr,<br>g./silver<br>mole | "Surface" Development |       |      | "Total" Development |       |      |
|-----------|-------------------------|---------------|---------------------------|-----------------------|-------|------|---------------------|-------|------|
|           |                         |               |                           | Relative<br>Speed     | Gamma | Fog  | Relative<br>Speed   | Gamma | Fog  |
| (l) ----- | All large (core) -----  | 135 min ----- | 6 -----                   | 74.0                  | 2.36  | 0.09 | 100                 | 2.16  | 0.10 |
| (m) ----- | 2:1 -----               | 260 min ----- | 6 -----                   | 6.7                   | 0.95  | 0.05 | 115                 | 1.68  | 0.16 |
| (n) ----- | 2:3 -----               | 260 min ----- | 10.8                      | 2.8                   | 0.46  | 0.05 | 170                 | 1.64  | 0.17 |

## EXAMPLE 5

The characteristic results obtained by covering a large emulsion grain (core) with a finer emulsion grain (shell) is also shown in this example. The emulsions used were similar to those described in Example 1 above, except that the ratio of the core emulsion to the shell emulsion was changed. The resulting covered grain (CG) emulsion contained 2 moles of large grain bromoiodide core to 3 moles of fine grain bromoiodide shell emulsion. The covered grain emulsion was coated on cellulose acetate film support, dried, and exposed in an intensity scale sensitometer, followed by development for 5 minutes in Developer B above, except that the developer contained no thiosulfate. Another CG sample was exposed in an identical manner and developed for 5 minutes in Developer D, which caused total development of the silver halide grains. The results are illustrated in the following table.

30  
35  
40  
45

exposure range. The numbers 150, 99, 191 and 175 appearing in the accompanying drawing are relative speed values for the respective coatings.

It was also surprising to discover that high intensity exposures of the CG emulsions of our invention to a Kodatron speed light increased the gammas substantially upon development for 5 minutes in Developer B above (except that it contained no thiosulfate), whereas the gamma of the basic core emulsion decreased under the same conditions. This is illustrated in the following table, which used emulsions similar to those described in Example 1 above, except that the ratio of core to shell emulsions was varied as illustrated in the table. As indicated, development was for 5 minutes in Developer B minus the thiosulfate.

Table V

| Coating<br>Number | Description                   | Surface Development |       |      | Total Development |       |      |
|-------------------|-------------------------------|---------------------|-------|------|-------------------|-------|------|
|                   |                               | Rel.<br>Speed       | Gamma | Fog  | Rel.<br>Speed     | Gamma | Fog  |
| (o) -----         | Control (core) emulsion ----- | 100                 | 2.00  | 0.07 | 129               | 2.16  | 0.12 |
| (p) -----         | CG emulsion; (2:3) -----      | 3.3                 | 0.30  | 0.05 | 229               | 1.51  | 0.18 |

The size of the covered grain emulsion grains depends upon the ratio of large to fine grains in the emulsion blends. As the amount of fine grain emulsion is increased, the volume of the covered grains increases and consequently the surface area. This is reflected in increased speeds as illustrated in the following table. These data were obtained exactly as described in Example 5, except that the ratio of large to fine grains was varied as illustrated in the table, and development was total development in Developer D.

Table VI

| CG large/fine grain ratio: | Relative speed |
|----------------------------|----------------|
| 1/0 -----                  | 100            |
| 2/1 -----                  | 132            |
| 1/1 -----                  | 159            |
| 2/3 -----                  | 186            |
| 1/3 -----                  | 251            |
| 1/7 -----                  | 398            |

60  
65  
70  
75

Table VII

| Coating<br>Number | Description<br>Core: Shell Ratio | Gamma                         |                      |
|-------------------|----------------------------------|-------------------------------|----------------------|
|                   |                                  | 1/25"<br>positive<br>exposure | Kodatron<br>exposure |
| (q) -----         | 2:1 -----                        | 0.95                          | 1.54                 |
| (r) -----         | 1:1 -----                        | 0.61                          | 1.28                 |
| (s) -----         | 2:3 -----                        | 0.46                          | 1.07                 |
| (t) -----         | 1:2 -----                        | 0.45                          | 1.05                 |
| (u) -----         | Core control -----               | 2.30                          | 1.98                 |

70  
75

It was also found that the surface latent image formed by direct X-ray exposure of the CG emulsion was more developable than that formed by 1 second exposure to visible light, even though the direct X-ray exposure was much less effective than visible light exposure on the normal core emulsion.

As indicated above, the CG emulsions of our invention can be spectrally sensitized using amounts of sensitizing dyes comparable to those used to sensitize normal surface sensitive emulsions of the same grain size, with the added advantage that much less blue desensitization is exhibited by the CG emulsions. It was also surprising to find that the CG emulsions exhibited improved incubation characteristics. The following table illustrates this improved incubation characteristic both with surface development for 5 minutes in Developer B minus the thiosulfate and for 5 minutes total development in Developer D. Emulsions similar to those in Example 1 were used, except that the core to shell ratio was varied as illustrated in the table. Data are given both for fresh coatings and coatings incubated for 2 weeks under constant humidity of about 55 percent and a temperature of about 120° F.

Table VIII

| Coating Number | Description (core/shell) | Surface Development |      |     |                 |      |     | Total Development |      |     |                 |      |     |
|----------------|--------------------------|---------------------|------|-----|-----------------|------|-----|-------------------|------|-----|-----------------|------|-----|
|                |                          | Fresh               |      |     | 2 wk. 120° Inc. |      |     | Fresh             |      |     | 2 wk. 120° Inc. |      |     |
|                |                          | Rel. Speed          | γ    | Fog | Rel. Speed      | γ    | Fog | Rel. Speed        | γ    | Fog | Rel. Speed      | γ    | Fog |
| (v)-----       | Core control-----        | 100                 | 2.40 | .16 | 240             | 1.98 | .48 | 102               | 2.10 | .21 | 214             | 1.70 | .54 |
| (w)-----       | CG (1:3)-----            | 1.9                 | .31  | .06 | 6.0             | .31  | .08 | 148               | 1.15 | .16 | 339             | 1.07 | .22 |
| (x)-----       | CG (2:3)-----            | 1.4                 | .24  | .06 | 9.7             | .31  | .10 | 170               | 1.33 | .31 | 276             | 1.22 | .42 |

It will be noted that the CG emulsions described above were considerably more stable toward fogging and loss of gamma during incubation.

If desired, the covered grain or CG emulsions of our invention can be further chemically sensitized or treated with sensitizing dyes or antifoggants according to methods well known to those skilled in the photographic art. For example, the CG emulsions of our invention can be chemically sensitized, spectrally sensitized, stabilized, treated with gelatin plasticizers, hardeners and the like, according to the methods described in Luckey and Hoppe U.S. application Serial No. 786,225, filed January 12, 1959 (now U.S. Patent 2,996,382, issued August 15, 1961).

In the preparation of the silver halide dispersions employed for preparing the silver halide emulsions of our invention, there may be employed as the dispersing agent for the silver halide in its preparation, gelatin or some other colloidal material, such as colloidal albumin, a polyacrylamide having a combined acrylamide content of 30-60% and a specific viscosity of 0.25-1.5 or an imidized polyacrylamide of like acrylimide content and viscosity as described in Lowe, Minsk and Kenyon U.S. Patent 2,541,474, issued February 13, 1951; zein as described in Lowe U.S. Patent 2,563,791, issued August 7, 1951; or a polymeric material which results from polymerizing a protein or a saturated acylated protein with a monomer having a vinyl group as described in Illingsworth, Dann and Gates U.S. Patent 2,852,383, issued September 16, 1958.

If desired, compatible mixtures of two or more of these colloids may be employed for dispersing the silver halide in its preparation. Combinations of antifoggants, sensitizers, hardeners, etc., may be used.

The photographic elements or CG emulsions described above may be used in diffusion transfer processes which utilize the undeveloped silver halide in the non-image areas of the negative to form a positive by dissolving the undeveloped silver halide and precipitating it on a receiving layer in close proximity to the silver halide emulsion layer. Such processes are described in Rott U.S. Patent 2,352,014, issued June 20, 1944, and Land U.S. Patents 2,584,029, issued January 29, 1952; 2,698-236, issued December 28, 1954, and 2,543,181, issued February 27, 1951; and Yackel et al. U.S. patent application Serial No. 586,705, filed May 23, 1956 (now U.S.

Patent 3,020,155, issued February 6, 1962). They may also be used in color transfer processes which utilize the diffusion transfer of an image-wise distribution of developer, coupler or dye, from a light-sensitive layer to a second layer, while the two layers are in close proximity to one another. Color processes of this type are described in Land U.S. Patents 2,559,643, issued July 10, 1951, and 2,698,798, issued January 4, 1955; Land and Rogers Belgian Patents 554,933 and 554,934, granted August 12, 1957; International Polaroid Belgian Patents 554,212, granted July 16, 1957 and 554,935, granted August 12, 1957; Yutzy U.S. Patent 2,756,142, issued July 24, 1956, and Whitmore and Mader U.S. patent application Serial No. 734,141, filed May 9, 1958 (now abandoned).

The addenda described above for use in conjunction with our emulsions can be employed in emulsions designed for X-ray photography, or in non-optically sensi-

tized emulsions, or orthochromatic- panchromatic- or infra-red sensitized emulsions. They can be added before or after sensitizing dyes are added. These addenda can also be used in emulsions designed for color photography, for example, emulsions containing color-forming compounds or couplers, or emulsions to be developed in solutions containing such couplers, or emulsions of the mixed-packet type, such as described in Godowsky U.S. Patent 2,698,794, issued January 4, 1955, etc.

The covered grain or CG emulsions of our invention can be treated with sufficient chemical sensitizer during the preparation to substantially completely fog the core emulsion component, and the resulting fogged internally sensitive grains used in the invention described in Luckey and Hoppe U.S. Patent No. 2,996,382, mentioned above. The CG emulsions of our invention are also useful in producing reversal films, such as those described in Fallesen U.S. Patent 2,497,875, issued February 21, 1950.

The invention has been described in detail with particular reference to preferred embodiments thereof, but it will be understood that the variations and modifications can be effected within the spirit and scope of the invention as described hereinabove and as defined in the appended claims.

What we claim as our invention and desire secured by Letters Patent of the United States is:

1. A light-sensitive photographic silver halide emulsion containing silver halide grains having high internal sensitivity, said grains comprising a central core of chemically sensitized silver halide and covering said central core an outer shell of silver halide having low surface activity, said outer shell of silver halide being substantially free of chemical sensitization.

2. A light-sensitive photographic silver halide emulsion as described in claim 1 wherein the central core of silver halide has been chemically sensitized with a labile sulfur compound and a gold salt.

3. A light-sensitive photographic silver halide emulsion as described in claim 1 wherein the silver halide of the central core and the outer shell contain not more than 10 mole percent of iodide and at least 90 mole percent bromide.

4. A photographic element comprising a flexible support and at least one light-sensitive photographic silver halide emulsion layer containing silver bromide grains

comprising a central core of chemically-sensitized silver bromide and a contiguous, outer shell of silver bromide which is chemically unsensitized.

5. A photographic elements comprising a support and at least one light-sensitive photographic silver halide emulsion layer containing silver halide grains containing not more than 10 mole percent of iodide and at least 90 mole percent bromide, said grains comprising a central core of chemically-sensitized silver bromoiodide and a contiguous, outer shell of unsensitized silver bromo-iodide.

6. A photographic element comprising a support and at least one light-sensitive photographic silver halide emulsion layer containing internally, sulfur-sensitized silver halide grains containing at least 90 mole percent silver bromide, said grains comprising a central core of sulfur-sensitized silver bromide containing at least 90 mole percent silver bromide ad a contiguous, outer shell of unsensitized silver bromide containing at least 90 mole percent silver bromide.

7. A photographic element according to claim 6 wherein in said silver halide contains at least 90 mole percent silver bromide and not more than 10 mole percent silver iodide.

8. A photographic element comprising a support and at least one light-sensitive photographic silver halide emulsion layer containing internally, gold-sensitized silver halide grains containing at least 90 mole percent silver bromide, said grain comprising a central core of gold-sensitized silver bromide containing at least 90 mole percent silver bromide and a contiguous, outer shell of unsensitized silver bromide containing at least 90 mole percent silver bromide.

9. A photographic element according to claim 8 wherein in said silver halide contains at least 90 mole percent silver bromide and not more than 10 mole percent silver iodide.

10. A process of preparing photographic silver halide

5  
10  
15  
20  
25  
30  
35

emulsions comprising a central core of chemically-sensitized grains and a shell over said core of chemically-unsensitized silver halide grains comprising digesting a mixture of chemically-sensitized silver halide grains having an average diameter of at least about  $0.8\mu$  together with unsensitized silver halide grains having an average diameter less than  $0.4\mu$  until said mixture has a single population of silver halide grains of substantially average uniform diameter sized grains.

11. A photographic element comprising a flexible support and at least one light-sensitive photographic silver halide emulsion layer containing silver bromide grains comprising a central core of sulfur and gold-sensitized silver bromide and a contiguous, outer shell of silver bromide which is chemically unsensitized.

12. A photographic element comprising a support and at least one light-sensitive photographic silver halide emulsion layer containing silver halide grains having high internal sensitivity, said grains comprising a central core of chemically sensitized silver halide and covering said central core an outer shell of silver halide having low surface activity, said outer shell of silver halide being substantially free of chemical sensitization.

13. A photographic element as defined in claim 12 wherein said central core of silver halide has been chemically sensitized with a labile sulfur compound and a gold salt.

#### References Cited by the Examiner

#### UNITED STATES PATENTS

|           |       |               |       |        |
|-----------|-------|---------------|-------|--------|
| 2,456,956 | 12/48 | Knott et al.  | ----- | 96—22  |
| 2,518,698 | 8/50  | Lowe et al.   | ----- | 96—107 |
| 2,974,628 | 8/60  | Fierke et al. | ----- | 96—22  |
| 3,046,134 | 7/62  | Dann et al.   | ----- | 96—110 |

NORMAN G. TORCHIN, *Primary Examiner.*

PHILIP E. MANGAN, *Examiner.*